

# UNITED STATES PATENT OFFICE.

CHARLES A. HUTTINGER, OF LAKEWOOD, OHIO, ASSIGNOR, BY MESNE ASSIGNMENTS, TO THE ACME ARTIFICIAL SILK COMPANY, OF CLEVELAND, OHIO, A CORPORATION OF OHIO.

## PROCESS OF PRODUCING LUSTROUS THREADS, ETC.

1,425,654.

Specification of Letters Patent. Patented Aug. 15, 1922.

No Drawing.

Application filed June 12, 1919. Serial No. 303,776.

To all whom it may concern:

Be it known that I, CHARLES A. HUTTINGER, a citizen of the United States, resident of Lakewood, county of Cuyahoga, and State of Ohio, have invented new and useful Improvements in Processes of Producing Lustrous Threads, Etc., of which the following is a specification, the principle of the invention being herein explained and the best mode in which I have contemplated applying that principle, so as to distinguish it from other inventions.

My invention relates to processes for producing lustrous threads, etc., from viscose. The invention contemplates an improvement upon the process for this purpose described in U. S. Letters Patent No. 836,452, issued November 20, 1906. The improvement, primarily, consists in producing threads of the character described, by means of forcing a viscose solution of certain characteristics hereinafter fully described through dies into a second or precipitating bath consisting of water and sodium bisulphate, said bath being used at a temperature of substantially seventy (70) degrees Fahrenheit and containing no free acid. The improvement, thus, resides in the ability to produce a product of the necessary qualities as regards its luster, strength and elasticity, without the necessity of using an acid in the precipitating bath and without the necessity of heating the latter above the usual working room temperature. This is accomplished both by the proportions of the ingredients which I utilize in making my viscose solution and in my methods of compounding same.

The following description sets forth in detail certain steps illustrating the method of carrying out my invention, such disclosed steps constituting, however, but one of the various ways in which the principle of the invention may be utilized.

In carrying out my improved process, I cut up a certain amount of wood pulp, one kilogram for instance, and then saturate the same with sodium hydroxide. The saturation is effected by a water solution of sodium hydroxide of substantially 1.17 specific gravity. The amount of sodium hydroxide which I use, for the stated amount of wood pulp, is substantially 515 grams, and the

amount of water utilized in making a solution of the specific gravity noted is substantially 2918 grams, which is a 15 per cent solution of sodium hydroxide. The treatment of the wood pulp with this sodium hydroxide solution continues for from one to five hours, preferably about one and a half hours. I then subject the wood pulp and sodium hydroxide water solution to great pressure, by means of a hydraulic press when treating comparatively large amounts, or by means of a screw press for small quantities, so that the material remaining on the press, i. e., the alkali cellulose, amounts to substantially 3 kilograms, when using the various amounts stated. Of these 3 kilograms, substantially 13.5 per cent is alkali, substantially 27 per cent is cellulose, and the remainder, 59.5 per cent, is water. I grind up these 3 kilograms of alkali cellulose remaining on the press, this alkali cellulose being a crumby material. I then subject the same to the action of substantially 325 grams of carbon bisulphide for about two hours. I then add water of substantially fifteen (15) times the amount of wood pulp originally utilized, or, as exactly as I have determined, 15.023 kilograms of water, the same being allowed to stand for substantially three hours. This comparatively large amount of water will dissolve some of the small amount of free soda in the alkali cellulose-carbon bisulphide mixture, so that the water is slightly alkaline. The resultant mixture is filtered during an aging period of about five days.

In making up the second or precipitating bath, I utilize, for the amounts entering into the first bath which have been noted, 1 kilogram of water and substantially 613 grams of sodium bisulphate. This results in substantially a saturated precipitating bath which is maintained at this standard throughout the precipitating action by the addition of necessary amounts of sodium bisulphate, the total additions for the proportions stated, being about 1.6 kilos. Sodium bisulphate is a by-product which can be bought comparatively cheaply. The viscose solution, comprised and compounded as above noted, is forced through suitable dies, as for instance, the openings in a spinneret, into the precipitating bath. A thread

of the character described and having all the desirable qualities in the proper degree, is the result. The entire operation is carried out at room temperatures, substantially 5 70° Fah.

My explanation of my ability to thus secure a satisfactory thread without the absence of free acid in the precipitating bath is that my method of compounding the viscose solution results in a saturation thereof 10 with sodium hydroxide without there being present in the solution thereafter a high percentage of free soda, which free soda must necessarily be neutralized out of the 15 solution to leave the cellulose for the thread. This neutralization is effected by the acid heretofore used. Thus, the lack of surplus hydroxide in my method obviates the necessity of free acid to neutralize such sodium hydroxide. The non-necessity of free 20 acid for the action of the precipitating bath is very beneficial, since free acid grasps or acts too quickly for the best results; whereas, the action of the sodium bisulphate is 25 very satisfactory.

I do not limit myself to the use of sodium bisulphate inasmuch as all soluble semi-neutral sulphates may be used, as well as combinations of those elements which result 30 in soluble semi-neutral sulphates.

What I claim is:

1. The method of producing threads of the character described, consisting in, saturating wood pulp with a solution of sodium hydroxide and water of a specific gravity of substantially 1.17; subjecting the mixture to pressure; adding carbon bisulphide to the resultant alkali cellulose; adding water; filtering; and then forcing the 35 resultant viscose solution through suitable dies into a precipitating bath comprised of a semi-neutral sulphate salt and water, said bath containing no free acid and being used at a temperature of substantially seventy 40 (70) degrees Fahrenheit.

2. The method of producing threads of the character described, consisting in, saturating wood pulp with a solution of sodium hydroxide and water of a specific gravity 45 of substantially 1.17; subjecting the mixture to pressure; adding carbon bisulphide to the resultant alkali cellulose; adding water; filtering; and then forcing the resultant viscose solution through suitable dies 50 into a precipitating bath comprised of sodium bisulphate and water, said bath containing no free acid and being used at a temperature of substantially seventy (70) degrees Fahrenheit.

3. The method of producing threads of the character described, consisting in, saturating wood pulp with a solution of sodium hydroxide and water of a specific gravity 55 of substantially 1.17; subjecting the mixture to pressure; adding carbon bisulphide to the

resultant alkali cellulose; adding water; filtering; and then forcing the resultant viscose solution through suitable dies into a precipitating bath comprised of a saturated solution of water and sodium bisulphate, 70 said bath containing no free acid and being used at a temperature of substantially seventy (70) degrees Fahrenheit.

4. The method of producing threads of the character described, consisting in, saturating wood pulp with a water solution of sodium hydroxide of substantially a specific gravity of 1.17, and subjecting the mixture of said wood pulp and said solution to great pressure so that the resultant alkali cellulose will equal substantially three times the amount of wood pulp utilized, and of which the cellulose will comprise substantially 75 27 per cent; grinding said alkali cellulose; adding carbon bisulphide thereto of substantially one-third the amount of the original wood pulp utilized; adding water of substantially fifteen times the amount of wood pulp originally utilized; filtering; and then forcing the resultant filtrate through dies 80 into a solution of sodium bisulphate and water, said last-named solution containing no free acid and being used at a temperature of substantially seventy (70) degrees 85 Fahrenheit.

5. The method of producing threads of the character described, consisting in, saturating wood pulp with a water solution of sodium hydroxide by treating the pulp with the solution for substantially one and a half 90 hours, said sodium hydroxide water solution being of substantially 1.17 specific gravity; subjecting the mixture of wood pulp and said solution to great pressure so that the resultant alkali cellulose will equal substantially 95 three times the amount of wood pulp originally utilized, of which amount the cellulose will comprise substantially 27 per cent; grinding said alkali cellulose; adding carbon bisulphide thereto of substantially one-third the amount of the wood pulp originally utilized; adding water of substantially fifteen times the amount of wood pulp originally utilized; filtering; and then forcing the resultant filtrate through dies into a solution of substantially six-tenths (.6) part sodium bisulphate and one (1) part water, said last-named solution containing no free acid and being used at a temperature of substantially seventy (70) degrees Fahrenheit.

6. The method of producing threads of the character described, consisting in, saturating one kilo of wood pulp with a sodium hydroxide water solution consisting of substantially 515 grams of sodium hydroxide 100 and 2918 grams of water, said treatment continuing for substantially one and a half hours; subjecting the mixture to great pressure, so that the resultant alkali cellulose will equal substantially 3 kilograms, of 105

which 13.5 per cent is combined alkali and free soda and 27 per cent is cellulose, grinding up the resultant alkali cellulose, and then subjecting the same for substantially 5 two hours to the action of 325 grams of carbon bisulphide; adding substantially 15 kilograms of water; filtering and aging for substantially five days; and then forcing the

resultant product through dies into a bath maintained at a strength of substantially one (1) part water and six-tenths (.6) part sodium bisulphate, said bath being used at a temperature of substantially seventy (70) degrees Fahrenheit.

Signed by me this 10th day of June, 1919.  
CHARLES A. HUTTINGER.